# EUROPEAN PATENT SPECIFICATION

(11) **EP 2 567 019 B1**
(45) Date of publication and mention of the grant of the patent: **05.03.2014**
(21) Application number: 11716943.3
(22) Date of filing: 02.05.2011
(51) Int. Cl.: D06M 15/05, D06M 15/09, D06M 15/564, D06N 3/14

(54) **PROCESS FOR THE COATING OF TEXTILES**
VERFAHREN ZUR BESCHICHTUNG VON GEWEBEN
PROCÉDÉ DE REVÊTEMENT DE TEXTILES

(30) Priority: 16.09.2010 EP 10177050; 07.05.2010 WO PCT/CN2010/000641
(43) Date of publication of application: 13.03.2013
(73) Proprietor: Bayer Intellectual Property GmbH, 40789 Monheim (DE)
(72) Inventor: IRNICH, Rolf, Shanghai 200123 (CN); ZHAO, Xuehui, Shanghai 200123 (CN)
(74) Representative: BIP Patents
(86) International application number: PCT/EP2011/056971
(87) International publication number: WO 2011/138284

(56) References cited:
- US-A1- 2004 121 113

## Description

The present invention relates to a process for the production of coated textiles in which a textile substrate is firstly brought into contact with an aqueous dispersion comprising at least one inorganic salt and at least one modified cellulose.

The production of synthetic leather by coating textiles with plastics has been known for some time. Synthetic leathers are employed, inter alia, as shoe upper materials, for articles of clothing, as bag-making material or in the upholstery sector, for example. Besides other plastics, such as PVC, the main coating material used here is polyurethane. The generally known principles of coating textiles with polyurethane are described in W. Schröer, Textilveredlung [Textile Finishing] 1987, 22 (12), 459-467. A description of the coagulation process is additionally found in "New Materials Permeable to Water Vapor", Harro Träubel, Springer Verlag, Berlin, Heidelberg, New York, 1999, ISBN 3-540-64946-8, pages 42 to 63.

The main processes used in the production of synthetic leather are the direct coating process, the transfer coating process (indirect coating) and the coagulation (wet) process. In contrast to the direct process, the coating in the transfer process is applied to a temporary support with a subsequent lamination step, in which the film is combined with the textile substrate and detached from the temporary support (release paper). The transfer process is preferably employed with textile substrates, which do not permit high tensile stresses during coating, or with open fabrics which are not particularly dense.

In the coagulation process, a textile substrate is usually coated with a solution comprising polyurethane in DMF. In a second step, the coated substrate is passed through DMF/water baths, where the proportion of water is increased stepwise. Precipitation of the polyurethane and formation of a microporous film occur here. Use is made here of the fact that DMF and water have excellent miscibility and DMF and water serve as a solvent/non-solvent pair for polyurethane. Coagulated polyurethane coatings are employed, in particular, for high-quality synthetic leather, since they have comparatively good breathing activity and a leather feel. The basic principle of the coagulation process is based on the use of a suitable solvent/nonsolvent pair for polyurethane. The great advantage of the coagulation process is that microporous, breathing-active synthetic leather having an excellent leather feel can be obtained. Examples are, for example, the synthetic leather brands Clarino® and Alcantara®. A disadvantage of the coagulation process is the necessity to use large amounts of DMF as an organic solvent. In order to minimize the exposure of employees to DMF emissions during production, additional design measures have to be taken, which represent a not inconsiderable increased outlay compared with simpler processes. Furthermore, it is necessary to dispose of or work up large amounts of DMF_{/}water mixtures. This is problematical since water and DMF form an azeotrope and can therefore only be separated by distillation with increased effort.

US2004/121113 already describes a solvent free process for the production of coated textiles, comprising the step of bringing a textile substrate into contact with an aqueous polyurethane dispersion, followed by a precipitation step. The polyurethane dispersion contains a modified cellulose as thickener and its pH is adjusted to about 8 to 10 using ammoniumhydroxide,

One object of the present invention was therefore to develop a process for the coating of textile substrates which still enables coated textiles having good properties, such as, for example, good feel, to be obtained without the need to employ toxicologically unacceptable solvents, such as, for example, DMF.

The object has been achieved by a process for the production of coated textiles, comprising at least the steps of
a) bringing a textile substrate into contact with an aqueous dispersion A comprising at least one inorganic salt and at least one modified cellulose,
b) bringing a textile substrate into contact with an aqueous dispersion B comprising polyurethane and
c) precipitation of the polyurethane in or on the textile substrate.

In step a), a textile substrate is brought into contact with an aqueous solution comprising at least one inorganic salt and at least one modified cellulose.

The inorganic salt is preferably a salt selected from the group comprising alkali metal salts and alkaline-earth metal salts. The inorganic salt is particularly preferably a salt selected from the group consisting of alkali metal halides, alkali metal phosphates, alkali metal nitrates, alkali metal sulfates, alkali metal carbonates, alkali metal hydrogen carbonates, alkaline-earth metal halides, alkaline-earth metal nitrates, alkaline-earth metal phosphates, alkaline-earth metal sulfates, alkaline-earth metal carbonates and alkaline-earth metal hydrogen carbonates. The inorganic salt is very particularly preferably sodium chloride, potassium chloride, sodium sulfate, sodium carbonate, potassium sulfate, potassium carbonate, sodium hydrogen carbonate, potassium hydrogen carbonate, magnesium chloride, magnesium sulfate, magnesium nitrate, calcium chloride, calcium nitrate or calcium sulfate. The inorganic salt is even more preferably calcium nitrate, magnesium nitrate, calcium chloride or magnesium chloride.

The inorganic salt is preferably present in dispersion A in an amount of 0.01 to 25 % by weight, particularly preferably in an amount of 0.5 to 15 % by weight, and very particularly preferably in an amount of 0.5 to 10 % by weight, based on the total amount of dispersion A.

The chemically modified cellulose is preferably a compound selected from the group consisting of alkylated celluloses, hydroxyalkylated celluloses and carboxyalkylated celluloses.

The chemically modified cellulose is particularly preferably a compound selected from the group consisting of methylcellulose, ethylcellulose, propylcellulose, hydroxymethylcellulose, hydroxyethylcellulose, hydroxymethylcellulose, hydroxypropylmethylcellulose, carboxymethylcellulose, carboxyethylcellulose and carboxypropylcellulose.

The chemically modified cellulose is very particularly preferably methylcellulose or ethylcellulose.

The modified cellulose is preferably present in dispersion A in an amount of 10 ppm to 5 % by weight, particularly preferably in an amount of 100 ppm to 3 % by weight, very particularly preferably in an amount of 400 ppm to 1.5 % by weight, based on the total amount of dispersion A.

The textile substrate is preferably brought into contact with an aqueous dispersion A at room temperature for a period of 2 to 4 minutes, particularly preferably 1 to 2 minutes, very particularly preferably 0.2 to 1 minute. For the purposes of the present invention, bringing into contact means partial or complete immersion, preferably complete immersion, in a dispersion or application of the dispersion by means of a hand coater, printing or spraying.

After being brought into contact with a dispersion A, the textile substrate is preferably passed through a wringer device consisting of two rollers in order to remove the excess dispersion A. The wringer device here should preferably be set in such a way that dispersion A remains in the textile substrate in an amount of 60 to 180 % by weight, particularly preferably 70 to 140 %, very particularly preferably 80 to 120 %, based on the weight per unit area of the substrate (liquor uptake), before the substrate is brought into contact with a dispersion B containing polyurethane. The textile substrate is preferably partially dried for a period of 2 to 10 minutes, particularly preferably 1 to 5 minutes, using air, infrared or hot cylinders before it can be brought into contact with a dispersion B containing polyurethane.

The polyurethane present in dispersion B is not particularly restricted so long as it is soluble in water, the term "polyurethane" also encompassing polyurethane-polyureas. A review of polyurethane (PUR) dispersions and processes therefor can be found in Rosthauser & Nachtkamp, "Waterbome Polyurethanes, Advances in Urethane Science and Technology", Vol. 10, pages 121-162 (1987). Suitable dispersions are also described, for example, in "Kunststoffhandbuch" [Plastics Handbook], Vol. 7, 2nd Edition, Hauser, pages 24 to 26.

Constituent components of dispersions B used in accordance with the invention may be the following:
1) Organic di- and/or polyisocyanates, such as, for example, tetramethylene diisocyanate, hexamethylene diisocyanate (HDI), 2-methylpentamethylene diisocyanate, 2,2,4-trimethylhexamethylene diisocyanate (THDI), dodecanemethylene diisocyanate, 1,4-diisocyanatocyclohexane, 3-isocyanatomethyl-3,3,5-trimethylcyclohexyl isocyanate (isophorone diisocyanate = IPDI), 4,4'-diisocyanatodicyclohexylmethane (Desmodur® W), 4,4'-diisocyanato-3,3'-dimethyldicyclohexylmethane, 4,4'-diisocyanato-2,2-dicyclohexylpropane, 1,4-diisocyanatobenzene, 2,4- or 2,6-diisocyanatotoluene or mixtures of these isomers, 4,4'-, 2,4- or 2,2'-diisocyanatodiphenylmethane or mixtures of these isomers, 4,4-, 2,4'- or 2,2'-diisocyanato-2,2-diphenylpropane-p-xylene diisocyanate and α,α,α',α'-tetramethyl-m- or -p-xylene diisocyanate (TMXDI), and mixtures consisting of these compounds. For the purposes of modification, small amounts of trimers, urethanes, biurets, allophanates or uretdiones of the above-mentioned diisocyanates can be used. MDI, Desmodur W, HDI and/or IPDI are particularly preferred.
2) Polyhydroxyl compounds having 1 to 8, preferably 1.7 to 3.5 hydroxyl groups per molecule and an (average) molecular weight of up to 16,000, preferably up to 4000. Low-molecular-weight polyhydroxyl compounds defined in each case, such as, for example, ethylene glycol, 1,2-, 1,3-propylene glycol, 1,4-butanediol, 1,6-hexanediol, neopentyl glycol, trimethylolpropane, glycerol, the product of the reaction of 1 hydrazine + 2 propylene glycol and oligomeric or polymeric hydroxyl compounds having molecular weights of 350 to 10,000, preferably 840 to 3000, can be considered.
   Relatively high-molecular-weight hydroxyl compounds include hydroxypolyesters, hydroxypolyethers, hydroxypolythioethers, hydroxypolyacetates, hydroxypolycarbonates and/or hydroxypolyester amides which are known per se in polyurethane chemistry, preferably those having average molecular weights of 350 to 4000, particularly preferably those having average molecular weights of 840 to 3000. Hydroxypolycarbonates and/or hydroxypolyethers are particularly preferred. When they are used, coagulates having particular stability to hydrolysis can be prepared.
3a) Ionic or potentially ionic hydrophilizing agents containing an acid group and/or an acid group in salt form and at least one isocyanate-reactive group, for example an OH or NH₂ group. Examples are the Na salt of ethylenediamine-β-ethylsulfonic acid (AAS salt solution), dimethylolpropionic acid (DMPA), dimethylolbutyric acid, hydroxypivalic acid or adducts of 1 mol of diamine, preferably isophoronediamine, and 1 mol of an α,β-unsaturated carboxylic acid, preferably acrylic acid.
3b) Nonionic hydrophilizing agents in the form of mono- and/or difunctional polyethylene oxide or polyethylene-propylene oxide alcohols having molecular weights of 300 to 5000. Particular preference is given to monohydroxyl-functional ethylene oxide/propylene oxide polyethers based on n-butanol having 35 to 85 % by weight of ethylene oxide units and molecular weights of 900 to 2500. A content of at least 3 % by weight, in particular at least 6 % by weight, of nonionic hydrophilizing agents is preferred.
4) Blocking agents for isocyanate groups, such as, for example, oximes (acetone oxime, butanone oxime or cyclohexanone oxime), secondary amines (diisopropylamine, dicyclohexylamine), NH-acidic heterocyclic substances (3,5-dimethylpyrazole, imidazole, 1,2,4-triazole), CH-acidic esters (C₁₋₄-alkyl malonates, acetic acid esters) or lactams (ε-caprolactam). Butanone oxime, diisopropylamine and 1,2,4-triazole are particularly preferred.
5) Polyamines as built-in chain extenders. These include, for example, the polyamines discussed under 6). The diamino-functional hydrophilizing agents discussed under 3a) are also suitable as chain extenders to be incorporated.
6) Polyamine crosslinking agents. These are preferably aliphatic or cycloaliphatic diamines, although it is also possible, if needed, to use trifunctional polyamines or polyfunctional polyamines in order to achieve specific properties. In general, it is possible to use polyamines containing additional functional groups, such as, for example, OH groups. The polyamine crosslinking agents, which are not incorporated into the polymer backbone at normal or slightly elevated ambient temperatures, for example 20 to 60 °C, are either admixed immediately during preparation of the reactive dispersions or at a subsequent point in time. Examples of suitable aliphatic polyamines are ethylenediamine, 1,2- and 1,3-propylenediamine, 1,4-tetramethylenediamine, 1,6-hexamethylenediamine, the isomer mixture of 2,2,4- and 2,4,4-trimethylhexamethylenediamine, 2-methylpentamethylenediamine and diethylenetriamine.

In a further preferred embodiment, dispersion B comprises at least one coagulant besides polyurethane. A coagulant is a salt or acid , for example ammonium salts of organic acids, which causes coagulation of the polyurethane under certain conditions, such as, for example, a particular temperature. These substances include an acid-generating chemical agent, i.e. a substance which is not an acid at room temperature, but becomes an acid after warming. Certain examples of such compounds include ethylene glycol diacetate, ethylene glycol formate, diethylene glycol formate, triethyl citrate, monostearyl citrate and an organic acid ester.

The coagulant is preferably present in the composition in an amount of 1 to 10 % by weight, based on the solids content of dispersion B.

The polyurethane present in dispersion B is preferably an anionic and/or nonionic hydrophilized polyurethane, which is obtainable by
A) the preparation of isocyanate-functional prepolymers from
   A1) organic polyisocyanates
   A2) polymeric polyols having number average molecular weights of 400 to 8000 g/mol, preferably 400 to 6000 g/mol and particularly preferably 600 to 3000 g/mol, and OH functionalities of 1.5 to 6, preferably 1.8 to 3, particularly preferably 1.9 to 2.1, and
   A3) optionally hydroxyl-functional compounds having molecular weights of 32 to 400 g/mol and
   A4) optionally isocyanate-reactive, anionic or potentially anionic and/or optionally nonionic hydrophilizing agents,
B) subsequent reaction of all or some of the free NCO groups thereof
   B1) optionally with amino-functional compounds having molecular weights of 32 to 400 g/mol and/or
   B2) isocyanate-reactive, preferably amino-functional, anionic or potentially anionic hydrophilizing agents
with chain extension, and dispersion of the resultant prepolymers in water before, during or after step B), where any potentially ionic groups present are converted into the ionic form by partial or complete reaction with a neutralizer.

In order to achieve anionic hydrophilization, it is necessary to carry out A4) and/or B2) using hydrophilizing agents which contain at least one group which is reactive to NCO groups, such as amino, hydroxyl or thiol groups, and in addition contain -COO- or -SO₃ or -PO₃²⁻ as anionic groups or fully or partially protonated acid forms thereof as potentially anionic groups.

Preferred aqueous, anionic polyurethane dispersions (I) have a low degree of hydrophilic anionic groups, preferably 0.1 to 15 milliequivalents per 100 g of solid resin.

In order to achieve good sedimentation stability, the number average particle size of the specific polyurethane dispersions is preferably less than 750 nm, particularly preferably less than 500 nm and very particularly preferably less than 400 nm, determined by means of laser correlation spectroscopy.

The ratio of NCO groups in the compounds of component A1) to NCO-reactive groups, such as amino, hydroxyl or thiol groups, in the compounds of components A2) to A4) during preparation of the NCO-functional prepolymer is 1.05 to 3.5, preferably 1.2 to 3.0, particularly preferably 1.3 to 2.5.

The amino-functional compounds in step B) are employed in such an amount that the equivalent ratio of isocyanate-reactive amino groups in these compounds to the free isocyanate groups in the prepolymer is 40 to 150 %, preferably between 50 and 125 %, particularly preferably between 60 and 120 %.

Suitable polyisocyanates of component A1) are the aromatic, araliphatic, aliphatic or cycloaliphatic polyisocyanates having an NCO functionality of 2 which are known per se to the person skilled in the art.

Examples of suitable polyisocyanates of this type are 1,4-butylene diisocyanate, 1,6-hexamethylene diisocyanate (HDI), isophorone diisocyanate (IPDI), 2,2,4- and/or 2,4,4-trimethylhexamethylene diisocyanate, the isomeric bis(4,4'-isocyanatocyclohexyl)methanes or mixtures thereof with any desired isomer content, 1,4-cyclohexylene diisocyanate, 1,4-phenylene diisocyanate, 2,4- and/or 2,6-tolylene diisocyanate, 1,5-naphthylene diisocyanate, 2,2'- and/or 2,4'- and/or 4,4'-diphenylmethane diisocyanate, 1,3- and/or 1,4-bis(2-isocyanatoprop-2-yl)-benzene (TMXDI), 1,3-bis(isocyanatomethyl)benzene (XDI), and alkyl 2,6-diisocyanato-hexanoates (lysine diisocyanates) containing C₁-C₈-alkyl groups.

Besides the above-mentioned polyisocyanates, it is also possible to employ proportionately modified diisocyanates having a uretdione, isocyanurate, urethane, allophanate, biuret, iminooxadiazinedione and/or oxadiazinetrione structure and unmodified polyisocyanates containing more than 2 NCO groups per molecule, for example 4-isocyanatomethyloctane 1,8-diisocyanate (nonane triisocyanate) or triphenylmethane 4,4',4"-triisocyanate.

These are preferably polyisocyanates or polyisocyanate mixtures of the above-mentioned type containing exclusively aliphatically and/or cycloaliphatically bonded isocyanate groups and having an average NCO functionality of the mixture of 2 to 4, preferably 2 to 2.6 and particularly preferably 2 to 2.4.

1,6-Hexamethylene diisocyanate, isophorone diisocyanate, the isomeric bis(4,4'-isocyanatocyclohexyl)methanes, and mixtures thereof, are particularly preferably employed in A1).

Polymeric polyols having a number average molecular weight Mₙ of 400 to 8000 g/mol, preferably 400 to 6000 g/mol and particularly preferably 600 to 3000 g/mol, are employed in A2). These preferably have an OH functionality of 1.5 to 6, particularly preferably 1.8 to 3, very particularly preferably 1.9 to 2.1.

Polymeric polyols of this type are the polyester polyols, polyacrylate polyols, polyurethane polyols, polycarbonate polyols, polyether polyols, polyester polyacrylate polyols, polyurethane polyacrylate polyols, polyurethane polyester polyols, polyurethane polyether polyols, polyurethane polycarbonate polyols and polyester polycarbonate polyols known per se in polyurethane coating technology. They can be employed individually or in any desired mixtures with one another in A2).

Polyester polyols of this type are the polycondensates, known per se, of di- and optionally tri- and tetraols and di- and optionally tri- and tetracarboxylic acids or hydroxycarboxylic acids or lactones. Instead of the free polycarboxylic acids, it is also possible to use the corresponding polycarboxylic anhydrides or corresponding polycarboxylates of lower alcohols for the preparation of the polyesters.

Examples of suitable diols are ethylene glycol, butylene glycol, diethylene glycol, triethylene glycol, polyalkylene glycols, such as polyethylene glycol, furthermore 1,2-propanediol, 1,3-propanediol, 1,3-butanediol, 1,4-butanediol, 1,6-hexanediol and isomers, neopentyl glycol or neopentyl glycol hydroxypivalate, where 1,6-hexanediol and isomers, neopentyl glycol and neopentyl glycol hydroxypivalate are preferred. In addition, it is also possible to employ polyols, such as trimethylolpropane, glycerol, erythritol, pentaerythritol, trimethylolbenzene or trishydroxyethyl isocyanurate.

Dicarboxylic acids which can be employed are phthalic acid, isophthalic acid, terephthalic acid, tetrahydrophthalic acid, hexahydrophthalic acid, cyclohexanedicarboxylic acid, adipic acid, azelaic acid, sebacic acid, glutaric acid, tetrachlorophthalic acid, maleic acid, fumaric acid, itaconic acid, malonic acid, suberic acid, 2-methylsuccinic acid, 3,3-diethylglutaric acid and/or 2,2-dimethylsuccinic acid. The corresponding anhydrides can also be used as acid source.

So long as the average functionality of the polyol to be esterified is > 2, monocarboxylic acids, such as benzoic acid and hexanecarboxylic acid, can also be used in addition.

Preferred acids are aliphatic or aromatic acids of the above-mentioned type. Particular preference is given to adipic acid, isophthalic acid and optionally trimellitic acid.

Hydroxycarboxylic acids which can be used concomitantly as reaction participants in the preparation of a polyester polyol containing terminal hydroxyl groups are, for example, hydroxycaproic acid, hydroxybutyric acid, hydroxydecanoic acid, hydroxystearic acid and the like. Suitable lactones are caprolactone, butyrolactone and homologs. Caprolactone is preferred.

Hydroxyl-containing polycarbonates, preferably polycarbonate diols, having number average molecular weights Mₙ of 400 to 8000 g/mol, preferably 600 to 3000 g/mol, can likewise be employed in A2). These are obtainable by reaction of carbonic acid derivatives, such as diphenyl carbonate, dimethyl carbonate or phosgene, with polyols, preferably diols. Examples of diols of this type are ethylene glycol, 1,2- and 1,3-propanediol, 1,3- and 1,4-butanediol, 1,6-hexanediol, 1,8-octanediol, neopentyl glycol, 1,4-bishydroxymethylcyclohexane, 2-methyl-1,3-propanediol, 2,2,4-trimethyl-1,3-pentanediol, dipropylene glycol, polypropylene glycols, dibutylene glycol, polybutylene glycols, bisphenol A and lactone-modified diols of the above-mentioned type.

The polycarbonate diol preferably comprises 40 to 100 % by weight of hexanediol, preferably 1,6-hexanediol, and/or hexanediol derivatives. Hexanediol derivatives of this type are based on hexanediol and, besides terminal OH groups, contain ester or ether groups. Derivatives of this type are obtainable by reaction of hexanediol with excess caprolactone or by etherification of hexanediol with itself to give di- or trihexylene glycol.

Instead of or in addition to pure polycarbonate diols, it is also possible to employ polyether polycarbonate diols in A2).

The hydroxyl-containing polycarbonates preferably have a linear structure.

Polyether polyols can likewise be employed in A2).

Suitable polyether polyols are, for example, the polytetramethylene glycol polyethers known per se in polyurethane chemistry, as obtainable by polymerization of tetrahydrofuran by means of cationic ring opening.

Likewise suitable polyether polyols are the products, known per se, of the addition of styrene oxide, ethylene oxide, propylene oxide, butylene oxides and/or epichlorohydrin onto di- or polyfunctional starter molecules. Polyether polyols based on the at least proportionate addition of ethylene oxide onto di- or polyfunctional starter molecules can also be employed as component A4) (nonionic hydrophilizing agents).

Suitable starter molecules which can be employed are all compounds known from the prior art, such as, for example, water, butyl diglycol, glycerol, diethylene glycol, trimethylolpropane, propylene glycol, sorbitol, ethylenediamine, triethanolamine, 1,4-butanediol. Preferred starter molecules are water, ethylene glycol, propylene glycol, 1,4-butanediol, diethylene glycol and butyl diglycol.

Particularly preferred embodiments of the polyurethane dispersions (I) comprise, as component A2), a mixture of polycarbonate polyols and polytetramethylene glycol polyols, where the proportion of polycarbonate polyols in this mixture is 20 to 80 % by weight and the proportion of polytetramethylene glycol polyols is 80 to 20 % by weight. A proportion of 30 to 75 % by weight of polytetramethylene glycol polyols and a proportion of 25 to 70 % by weight of polycarbonate polyols are preferred. A proportion of 35 to 70 % by weight of polytetramethylene glycol polyols and a proportion of 30 to 65 % by weight of polycarbonate polyols are particularly preferred, in each case with the proviso that the sum of the per cent by weight of the polycarbonate polyols and polytetramethylene glycol polyols is 100 % and the proportion of the sum of the polycarbonate polyols and polytetramethylene glycol polyether polyols in component A2) is at least 50 % by weight, preferably 60 % by weight and particularly preferably at least 70 % by weight.

The compounds of component A3) have molecular weights of 62 to 400 g/mol.

Polyols in the said molecular weight range having up to 20 carbon atoms, such as ethylene glycol, diethylene glycol, triethylene glycol, 1,2-propanediol, 1,3-propanediol, 1,4-butanediol, 1,3-butylene glycol, cyclohexanediol, 1,4-cyclohexanedimethanol, 1,6-hexanediol, neopentyl glycol, hydroquinone dihydroxyethyl ether, bisphenol A (2,2-bis(4-hydroxyphenyl)propane), hydrogenated bisphenol A (2,2-bis(4-hydroxycyclohexyl)propane), trimethylolpropane, glycerol, pentaerythritol, and any desired mixtures thereof with one another, can be employed in A3).

Also suitable are ester diols in the said molecular weight range, such as α-hydroxybutyl-ε-hydroxycaproic acid esters, ω-hydroxyhexyl-γ-hydroxybutyric acid esters, β-hydroxyethyl adipate or β-hydroxyethyl terephthalate.

Furthermore, monofunctional, isocyanate-reactive, hydroxyl-containing compounds can also be employed in A3). Examples of monofunctional compounds of this type are ethanol, n-butanol, ethylene glycol monobutyl ether, diethylene glycol monomethyl ether, ethylene glycol monobutyl ether, diethylene glycol monobutyl ether, propylene glycol monomethyl ether, dipropylene glycol monomethyl ether, tripropylene glycol monomethyl ether, dipropylene glycol monopropyl ether, propylene glycol monobutyl ether, dipropylene glycol monobutyl ether, tripropylene glycol monobutyl ether, 2-ethylhexanol, 1-octanol, 1-dodecanol, 1-hexadecanol.

Preferred compounds of component A3) are 1,6-hexanediol, 1,4-butanediol, neopentyl glycol and trimethylolpropane.

Anionically or potentially anionically hydrophilizing compounds of component A4) are taken to mean all compounds which contain at least one isocyanate-reactive group, such as a hydroxyl group, and at least one functionality, such as, for example, -COO-M⁺, -SO₃⁻M⁺, -PO(O⁻M⁺)₂, where M⁺ is, for example, a metal cation, H⁺, NH₄⁺, NHR₃⁺, where R may in each case be a C₁-C₁₂-alkyl, C₅-C₆-cycloalkyl and/or C₂-C₄-hydroxyalkyl radical, which enters into a pH-dependent dissociation equilibrium on interaction with aqueous media and may in this way be negatively charged or neutral. Suitable anionically or potentially anionically hydrophilizing compounds are mono- and dihydroxycarboxylic acids, mono- and dihydroxysulfonic acids, and mono- and dihydroxyphosphonic acids, and salts thereof. Examples of anionic or potentially anionic hydrophilizing agents of this type are dimethylolpropionic acid, dimethylolbutyric acid, hydroxypivalic acid, malic acid, citric acid, glycolic acid, lactic acid and the propoxylated adduct of 2-butenediol and NaHSO₃, as described in DE-A 2 446 440, pages 5 - 9, formulae I-III. Preferred anionic or potentially anionic hydrophilizing agents of component A4) are those of the above-mentioned type which contain carboxylate or carboxylic acid groups and/or sulfonate groups.

Particularly preferred anionic or potentially anionic hydrophilizing agents A4) are those which contain carboxylate or carboxylic acid groups as ionic or potentially ionic groups, such as dimethylolpropionic acid, dimethylolbutyric acid and hydroxypivalic acid, or salts thereof.

Suitable nonionically hydrophilizing compounds of component A4) are, for example, polyoxyalkylene ethers which contain at least one hydroxyl or amino group, preferably at least one hydroxyl group.

Examples are the monohydroxyl-functional polyalkylene oxide polyether alcohols containing on statistical average 5 to 70, preferably 7 to 55 ethylene oxide units per molecule, as are accessible in a manner known per se by alkoxylation of suitable starter molecules (for example in Ullmanns Encyclopädie der technischen Chemie [Ullmann's Encyclopedia of Industrial Chemistry], 4th Edition, Volume 19, Verlag Chemie, Weinheim pp. 31-38).

These are either pure polyethylene oxide ethers or mixed polyalkylene oxide ethers, which contain at least 30 mol %, preferably at least 40 mol %, based on all alkylene oxide units present, of ethylene oxide units.

Particularly preferred nonionic compounds are monofunctional mixed polyalkylene oxide polyethers which contain 40 to 100 mol % of ethylene oxide units and 0 to 60 mol % of propylene oxide units.

Suitable starter molecules for nonionic hydrophilizing agents of this type are saturated monoalcohols, such as methanol, ethanol, n-propanol, isopropanol, n-butanol, isobutanol, sec-butanol, the isomeric pentanols, hexanols, octanols and nonanols, n-decanol, n-dodecanol, n-tetradecanol, n-hexadecanol, n-octadecanol, cyclohexanol, the isomeric methylcyclohexanols or hydroxymethylcyclohexane, 3-ethyl-3-hydroxymethyloxetane or tetrahydrofurfuryl alcohol, diethylene glycol monoalkyl ethers, such as, for example, diethylene glycol monobutyl ether, unsaturated alcohols, such as allyl alcohol, 1,1-dimethylallyl alcohol or oleyl alcohol, aromatic alcohols, such as phenol, the isomeric cresols or methoxyphenols, araliphatic alcohols, such as benzyl alcohol, anisalcohol or cinnamyl alcohol, secondary monoamines, such as dimethylamine, diethylamine, dipropylamine, diisopropylamine, dibutylamine, bis(2-ethylhexyl)amine, N-methyl- and N-ethylcyclohexylamine or dicyclohexylamine, and heterocyclic secondary amines, such as morpholine, pyrrolidine, piperidine or 1H-pyrazole. Preferred starter molecules are saturated monoalcohols of the above-mentioned type. Diethylene glycol monobutyl ether or n-butanol is particularly preferably used as starter molecule.

Alkylene oxides which are suitable for the alkoxylation reaction are, in particular, ethylene oxide and propylene oxide, which can be employed in any desired sequence or also as a mixture in the alkoxylation reaction.

Di- or polyamines, such as 1,2-ethylenediamine, 1,2- and 1,3-diaminopropane, 1,4-diamino-butane, 1,6-diaminohexane, isophoronediamine, isomer mixture of 2,2,4- and 2,4,4-trimethylhexamethylenediamine, 2-methylpentamethylenediamine, diethylenetriamine, triaminononane, 1,3- and 1,4-xylylenediamine, α,α,α',α'-tetramethyl-1,3- and -1,4-xylylenediamine and 4,4-diaminodicyclohexylmethane and/or dimethylethylenediamine, can be employed as component B1). It is likewise possible to use hydrazine or hydrazides, such as adipohydrazide. Preference is given to isophoronediamine, 1,2-ethylenediamine, 1,4-diaminobutane, hydrazine and diethylenetriamine.

In addition, compounds which, besides a primary amino group, also contain secondary amino groups or, besides an amino group (primary or secondary), also contain OH groups can also be employed as component B1). Examples thereof are primary/secondary amines, such as diethanolamine, 3-amino-1-methylaminopropane, 3-amino-1-ethylaminopropane, 3-amino-1-cyclohexylaminopropane, 3-amino-1-methylaminobutane, alkanolamines, such as N-amino-ethylethanolamine, ethanolamine, 3-aminopropanol, neopentanolamine.

Furthermore, monofunctional isocyanate-reactive amino compounds, such as, for example, methylamine, ethylamine, propylamine, butylamine, octylamine, laurylamine, stearylamine, isononyloxypropylamine, dimethylamine, diethylamine, dipropylamine, dibutylamine, N-methylaminopropylamine, diethyl(methyl)aminopropylamine, morpholine, piperidine, or suitable substituted derivatives thereof, amidoamines made from diprimary amines and monocarboxylic acids, monoketimes of diprimary amines, primary/tertiary amines, such as N,N-dimethylaminopropylamine, can also be employed as component B1).

Preferred compounds of component B1) are 1,2-ethylenediamine, 1,4-diaminobutane and isophoronediamine.

Anionically or potentially anionically hydrophilizing compounds of component B2) are taken to mean all compounds which contain at least one isocyanate-reactive group, preferably an amino group, and at least one functionality, such as, for example, -COO⁻M⁺, -SO₃⁻M⁺, -PO(O⁻M⁺)₂, where M⁺ is, for example, a metal cation, H⁺, NH₄⁺, NHR₃⁺, where R may in each case be a C₁-C₁₂-alkyl radical, C₅-C₆-cycloalkyl radical and/or C₂-C₄-hydroxyalkyl radical, which enters into a pH-dependent dissociation equilibrium on interaction with aqueous media and may in this way be negatively charged or neutral.

Suitable anionically or potentially anionically hydrophilizing compounds are mono- and diaminocarboxylic acids, mono- and diaminosulfonic acids and mono- and diaminophosphonic acids, and salts thereof. Examples of anionic or potentially anionic hydrophilizing agents of this type are N-(2-aminoethyl)-β-alanine, 2-(2-aminoethylamino)-ethanesulfonic acid, ethylenediaminepropyl- or -butylsulfonic acid, 1,2- or 1,3-propylenediamine-β-ethylsulfonic acid, glycine, alanine, taurine, lysine, 3,5-diaminobenzoic acid and the product of the addition reaction of IPDA and acrylic acid (EP-A 0 916 647, Example 1). Furthermore, cyclohexylaminopropanesulfonic acid (CAPA), which is known from WO-A 01/88006, can be used as an anionic or potentially anionic hydrophilizing agent.

Preferred anionic or potentially anionic hydrophilizing agents of component B2) are those of the above-mentioned type which contain carboxylate or carboxylic acid groups and/or sulfonate groups, such as the salts of N-(2-aminoethyl)-β-alanine, of 2-(2-aminoethylamino)ethanesulfonic acid or of the product of the addition reaction of IPDA and acrylic acid (EP-A 0 916 647, Example 1).

The hydrophilization can also be carried out using mixtures of anionic or potentially anionic hydrophilizing agents and nonionic hydrophilizing agents.

In a preferred embodiment for the preparation of the specific polyurethane dispersions, components A1) to A4) and B1) to B2) are employed in the following amounts, where the individual amounts always add up to 100 % by weight:
5 to 40 % by weight of component A1),
55 to 90 % by weight of A2),
0.5 to 20 % by weight of the sum of components A3) and B1),
0.1 to 25 % by weight of the sum of components A4) and B2), where 0.1 to 5 % by weight of anionic or potentially anionic hydrophilizing agents from A4) and/or B2) are used, based on the total amounts of components A1) to A4) and B1) to B2).

In a particularly preferred embodiment for the preparation of the specific polyurethane dispersions, components A1) to A4) and B1) to B2) are employed in the following amounts, where the individual amounts always add up to 100 % by weight:
5 to 35 % by weight of component A1),
60 to 90 % by weight of A2),
0.5 to 15 % by weight of the sum of components A3) and B1),
0.1 to 15 % by weight of the sum of components A4) and B2), where 0.2 to 4 % by weight of anionic or potentially anionic hydrophilizing agents from A4) and/or B2) are used, based on the total amounts of components A1) to A4) and B1) to B2).

In a very particularly preferred embodiment for the preparation of the specific polyurethane dispersions, components A1) to A4) and B1) to B2) are employed in the following amounts, where the individual amounts always add up to 100 % by weight:
10 to 30 % by weight of component A1),
65 to 85 % by weight of A2),
0.5 to 14 % by weight of the sum of components A3) and B1),
0.1 to 13.5 % by weight of the sum of components A4) and B2), where 0.5 to 3.0 % by weight of anionic or potentially anionic hydrophilizing agents from A4) and/or B2) are used, based on the total amounts of components A1) to A4) and B1) to B2).

The preparation of the anionically hydrophilized polyurethane dispersions (I) can be carried out in one or more steps in a homogeneous or multistep reaction, some in the disperse phase. After complete or partial polyaddition from A1) to A4), a dispersion, emulsification or dissolution step is carried out. If desired, a further polyaddition or modification in the disperse phase is subsequently carried out.

All processes known from the prior art, such as, for example, the prepolymer mixing process, acetone process or melt dispersal process, can be used here. The acetone process is preferably used.

For preparation by the acetone process, all or some of constituents A2) to A4) and the polyisocyanate component A1) are usually initially introduced for the preparation of an isocyanate-functional polyurethane prepolymer and optionally diluted with a solvent which is miscible with water, but inert to isocyanate groups and heated to temperatures in the range from 50 to 120 °C. In order to accelerate the isocyanate addition reaction, the catalysts known in polyurethane chemistry can be employed.

Suitable solvents are the conventional aliphatic, keto-functional solvents, such as acetone, 2-butanone, which can be added not only at the beginning of the preparation, but, if desired, can also partly be added later. Preference is given to acetone and 2-butanone.

Other solvents, such as xylene, toluene, cyclohexane, butyl acetate, methoxypropyl acetate, N-methylpyrrolidone, N-ethylpyrrolidone, solvents containing ether or ester units, may additionally be employed and distilled off in full or part or, in the case of N-methylpyrrolidone, N-ethylpyrrolidone, remain completely in the dispersion. However, other solvents apart from the conventional aliphatic, keto-functional solvents are preferably not used.

Any constituents of A1) to A4) which have not yet been added at the beginning of the reaction are subsequently metered in.

In the preparation of the polyurethane prepolymer from A1) to A4), the molar ratio of isocyanate groups to isocyanate-reactive groups is 1.05 to 3.5, preferably 1.2 to 3.0, particularly preferably 1.3 to 2.5.

The conversion of components A1) to A4) into the prepolymer is carried out in part or full, but preferably in full. Thus, polyurethane prepolymers which contain free isocyanate groups are obtained in the solid state or in solution.

In the neutralization step for the partial or complete conversion of potentially anionic groups into anionic groups, bases, such as tertiary amines, for example trialkylamines having 1 to 12 C atoms, preferably 1 to 6 C atoms, particularly preferably 2 to 3 C atoms, in each alkyl radical or alkali metal bases, such as the corresponding hydroxides, are employed.

Examples thereof are trimethylamine, triethylamine, methyldiethylamine, tripropylamine, N-methylmorpholine, methyldiisopropylamine, ethyldiisopropylamine and diisopropylethylamine. The alkyl radicals may also carry, for example, hydroxyl groups, as in the case of the dialkylmonoalkanolamines, alkyldialkanolamines and trialkanolamines. Neutralizers which can be employed, if desired, are also inorganic bases, such as aqueous ammonia solution or sodium hydroxide or potassium hydroxide.

Preference is given to ammonia, triethylamine, triethanolamine, dimethylethanolamine or diisopropylethylamine, as well as sodium hydroxide and potassium hydroxide, particularly preferably sodium hydroxide and potassium hydroxide.

The molar amount of the bases is 50 to 125 mol %, preferably between 70 and 100 mol %, of the molar amount of the acid groups to be neutralized. The neutralization can also be carried out simultaneously with the dispersion if the dispersion water already comprises the neutralizer.

In a further process step, the resultant prepolymer is subsequently dissolved, if this has not already taken place or has only taken place in part, with the aid of aliphatic ketones, such as acetone or 2-butanone.

In the chain extension in step B), NH₂- and/or NH-functional components are reacted in part or full with the remaining isocyanate groups of the prepolymer. The chain extension/termination is preferably carried out before the dispersion in water.

For the chain termination, amines B1) containing an isocyanate-reactive group, such as methylamine, ethylamine, propylamine, butylamine, octylamine, laurylamine, stearylamine, isononyloxypropylamine, dimethylamine, diethylamine, dipropylamine, dibutylamine, N-methylaminopropylamine, diethyl(methyl)aminopropylamine, morpholine, piperidine, or suitable substituted derivatives thereof, amidoamines made from diprimary amines and monocarboxylic acids, monoketimes of diprimary amines, primary/tertiary amines, such as N,N-dimethylaminopropylamine, are usually used.

If the partial or complete chain extension is carried out using anionic or potentially anionic hydrophilizing agents corresponding to definition B2) containing NH₂ or NH groups, the chain extension of the prepolymers is preferably carried out before the dispersion.

The aminic components B1) and B2) can optionally be employed in water- or solvent-diluted form in the process according to the invention, individually or in mixtures, where any sequence of addition is in principle possible.

If water or organic solvents are used concomitantly as diluents, the diluent content in the component employed in B) for chain extension is preferably 70 to 95 % by weight.

The dispersion is preferably carried out after the chain extension. To this end, the dissolved and chain-extended polyurethane polymer is either introduced into the dispersion water, optionally with high shear, such as, for example, vigorous stirring, or conversely the dispersion water is stirred into the chain-extended polyurethane polymer solutions. The water is preferably added to the dissolved chain-extended polyurethane polymer.

The solvent still present in the dispersions after the dispersion step is usually subsequently removed by distillation. Removal during the dispersion is likewise possible.

The residual content of organic solvents in the polyurethane dispersions (I) is typically less than 1.0 % by weight, based on the entire dispersion.

The pH of the polyurethane dispersions (I) which are essential to the invention is typically less than 9.0, preferably less than 8.5, particularly preferably less than 8.0 and very particularly preferably 6.0 to 7.5.

The solids content of the polyurethane dispersions (I) is 40 to 70 % by weight, preferably 50 to 65 % by weight, particularly preferably 55 to 65 % by weight.

In a further preferred embodiment, dispersion B likewise comprises coagulants (II) besides anionically hydrophilized polyurethane.

Coagulants (II) which can be employed in the compositions are all organic compounds containing at least 2 cationic groups, preferably all known cationic flocculants and precipitants from the prior art, such as cationic homopolymers or copolymers of salts of poly[2-(N,N,N-trimethylamino)ethyl acrylate], of polyethyleneimine, of poly[N-(dimethylamino-methyl)-acrylamide], of substituted acrylamides, of substituted methacrylamides, of N-vinylformamide, ofN-vinylacetamide, of N-vinylimidazole, of 2-vinylpyridine or of 4-vinylpyridine.

Preferred coagulants (II) are cationic copolymers of acrylamide which contain structural units of the general formula (2), particularly preferably cationic copolymers of acrylamide which contain structural units of the formula (1) and those of the general formula (2): where
- R: is C=O, -COO(CH₂)₂- or -COO(CH₂)₃- and
- X⁻: is a halide ion, preferably chloride.

The cationic coagulant (II) employed is particularly preferably a polymer of this type having a number average molecular weight of 500,000 to 50,000,000 g/mol.

Coagulants (II) of this type are marketed, for example, under the trade name Praestol^{®} (Degussa Stockhausen, Krefeld, DE) as flocculants for sewage sludges. Preferred coagulants of the Praestol^{®} type are Praestol^{®} K111L, K122L, K133L, BC 270L, K 144L, K 166L, BC 55L, 185K, 187K, 190K, K222L, K232L, K233L, K234L, K255L, K332L, K 333L, K 334L, E 125, E 150, and mixtures thereof. Very particularly preferred coagulants are Praestol^{®} 185K, 187K and 190K, and mixtures thereof.

Dispersion B preferably comprises at least one pigment.

The manner in which the precipitation in or on the textile substrate is accomplished depends to a large extent on the chemical composition of the dispersion B used in accordance with the invention and in particular on the type of coagulant, if present. For example, the precipitation can be carried out by evaporation coagulation or by salt, acid or electrolyte coagulation.

In general, the precipitation is achieved by an increase in temperature. For example, the textile substrate can be subjected to brief heat treatment with steam, for example at 100 to 110 °C for 1 to 10 s. This is particularly preferred if ammonium salts or organic acids are used as coagulant. If, on the other hand, the above-mentioned acid-generating chemicals are used as coagulant, the precipitation is preferably carried out as described in US 5,916,636, US 5,968,597, US 5,952,413 and US 6,040,393.

Alternatively, the coagulation is caused by dipping into a salt solution. The coagulation is preferably carried out using an inorganic salt selected from the group consisting of alkali metal salts and alkaline-earth metal salts. The inorganic salt is particularly preferably a salt selected from the group consisting of alkali metal halides, alkali metal nitrates, alkali metal phosphates, alkali metal sulfates, alkali metal carbonates, alkali metal hydrogen carbonates, alkaline-earth metal halides, alkaline-earth metal phosphates, alkaline-earth metal nitrates, alkaline-earth metal sulfates, alkaline-earth metal carbonates and alkaline-earth metal hydrogen carbonates. The inorganic salt is very particularly preferably sodium chloride, potassium chloride, sodium sulfate, sodium carbonate, potassium sulfate, potassium carbonate, sodium hydrogen carbonate, potassium hydrogen carbonate, magnesium chloride, magnesium sulfate, calcium chloride or calcium sulfate. The inorganic salt is still more preferably calcium chloride or magnesium chloride.

The inorganic salt is preferably present in the salt solution in an amount of 1 to 25 % by weight, particularly preferably in an amount of 1 to 15 % by weight, very particularly preferably in an amount of 1 to 10 % by weight, based on the total amount of salt solution.

After the precipitation in step c), further steps, such as drying or condensation, are carried out if necessary.

The textile substrate employed is preferably a woven fabric, knitted fabric or nonwoven based on natural and/or synthetic fibers. The textile substrate is particularly preferably a nonwoven (staple fiber nonwoven, microfiber nonwoven or the like).

The textile substrate can preferably be built up from fibers of polyester, nylon (6 or 6,6), cotton, polyester/cotton blends, wool, ramie, spandex, glass, thermoplastic polyurethane (TPU), thermoplastic olefins (TPO) or the like. The textile substrate can have a linked/mesh-like (knitted), woven or nonwoven construction.

The textile substrate can be treated with dyes, colorants, pigments, UV absorbers, plasticizers, soil redeposition agents, lubricants, antioxidants, flame inhibitors, rheology agents and the like, either before coating or thereafter, but there is a preference for such additions before coating.

If a defined nonwoven fabric is impregnated with an elastomer polymer and coagulated, and a normal coloring process is subsequently carried out, a suede-like synthetic leather having good color development properties is obtained.

The present invention therefore furthermore relates to a coated textile, preferably synthetic leather, obtained by the process according to the invention.

### Examples

Dispersion A has the following composition:

Dispersion B1 for salt coagulation has the following composition:

The process for the preparation of the coated textile using salt coagualtion is described in Fig. 1.

Dispersion B2 for heat coagulation has the following composition:

The process for the preparation of the coated textile using heat coagualtion is described in Fig. 2.

Substrates which have been subjected to the process without the bringing into contact with dispersion A as described had a very hard and stiff feel. By contrast, substrates which were treated in accordance with the invention exhibited a pleasantly soft, round feel. On subsequent coating of the resultant substrates, considerable differences were likewise apparent between the substrates treated with dispersion A and the untreated substrates, such that the fall of the folds (folding) appeared sharp and/or blistered in the case of the untreated coagulant. The substrate treated in accordance with the invention exhibited round, optically perfect folding.

## Claims

1. Process for the production of coated textiles,
comprising at least the steps of
a) bringing a textile substrate into contact with an aqueous dispersion A comprising at least one inorganic salt and at least one modified cellulose,
b) bringing a textile substrate into contact with an aqueous dispersion B comprising polyurethane and
c) precipitation of the polyurethane in or on the textile substrate.

2. Process according to Claim 1, where the inorganic salt is a salt selected from the group consisting of alkali metal salts and alkaline-earth metal salts.

3. Process according to Claim 2, where the alkali metal salt is a salt selected from the group consisting of alkali metal halides, alkali metal nitrates, alkali metal phosphates, alkali metal sulfates, alkali metal carbonates and alkali metal hydrogen carbonates.

4. Process according to Claim 2, where the allcaline-earth metal salt is a salt selected from the group consisting of alkaline-earth metal halides, alkaline-earth metal nitrates, alkaline-earth metal phosphates, alkaline-earth metal sulfates, alkaline-earth metal carbonates and alkaline-earth metal hydrogen carbonates.

5. Process according to Claim 1, where the inorganic salt is present in dispersion A in an amount of 0.01 to 25 % by weight, based on the total amount of dispersion A.

6. Process according to Claim 1, where the modified cellulose is a compound selected from the group consisting of methylcellulose, ethylcellulose, propylcellulose, hydroxymethylcellulose, hydroxyethylcellulose, hydroxypropylcellulose, hydroxypropylmethylcellulose, carboxymethylcellulose, carboxyethylcellulose and carboxypropylcellulose.

7. Process according to Claim 1, where the modified cellulose is present in dispersion A in an amount of 10 ppm to 5 % by weight, based on the total amount of dispersion A.

8. Process according to Claim 1, **characterized in that** the textile substrate employed is a woven fabric, knitted fabric or nonwoven based on natural and/or synthetic fibers.

9. Process according to Claim 1, **characterized in that** the polyurethane is precipitated in step c) in a bath containing water or on use of a temperature in the range from 80 to 120 °C.

10. Coated textile obtainable by a process according to Claims 1 to 9.

11. Coated textile according to Claim 10, **characterized in that** the coated textile is synthetic leather.

## Patentansprüche

1. Verfahren zur Herstellung von beschichteten Textilien, das mindestens folgende Schritte umfasst:
a) Inberührungbringen eines textilen Substrats mit einer wässrigen Dispersion A, die mindestens ein anorganisches Salz und mindestens eine modifizierte Zellulose enthält,
b) Inberührungbringen eines textilen Substrats mit einer wässrigen Dispersion B, die Polyurethan enthält, und
c) Ausfällen des Polyurethans in oder auf dem textilen Substrat.

2. Verfahren nach Anspruch 1, bei dem es sich bei dem anorganischen Salz um ein Salz aus der Gruppe bestehend aus Alkalimetallsalzen und Erdalkalimetallsalzen handelt.

3. Verfahren nach Anspruch 2, bei dem es sich bei dem Alkalimetallsalz um ein Salz aus der Gruppe bestehend aus Alkalimetallhalogeniden, Alkalimetallnitraten, Alkalimetallphosphaten, Alkalimetallsulfaten, Alkalimetallcarbonaten und Alkalimetallhydrogencarbonaten handelt.

4. Verfahren nach Anspruch 2, bei dem es sich bei dem Erdalkalimetallsalz um ein Salz aus der Gruppe bestehend aus Erdalkalimetallhalogeniden, Erdalkalimetallnitraten, Erdalkalimetallphosphaten, Erdalkalimetallsulfaten, Erdalkalimetallcarbonaten und Erdalkalimetallhydrogencarbonaten handelt.

5. Verfahren nach Anspruch 1, bei dem das anorganische Salz in Dispersion A in einer Menge von 0,01 bis 25 Gew.-%, bezogen auf die Gesamtmenge von Dispersion A, vorliegt.

6. Verfahren nach Anspruch 1, bei dem es sich bei der modifizierten Cellulose um eine Verbindung aus der Gruppe bestehend aus Methylcellulose, Ethylcellulose, Propylcellulose, Hydroxymethylcellulose, Hydroxyethylcellulose, Hydroxypropylcellulose, Hydroxypropylmethylcellulose, Carboxymethylcellulose, Carboxyethylcellulose und Carboxypropylcellulose handelt.

7. Verfahren nach Anspruch 1, bei dem die modifizierte Cellulose in Dispersion A in einer Menge von 10 Gew.-ppm bis 5 Gew.-%, bezogen auf die Gesamtmenge von Dispersion A, vorliegt.

8. Verfahren nach Anspruch 1, **dadurch gekennzeichnet, dass** es sich bei dem eingesetzten textilen Substrat um ein Gewebe, ein Gewirk oder einen Vliesstoff auf Basis von natürlichen und/oder synthetischen Fasern handelt.

9. Verfahren nach Anspruch 1, **dadurch gekennzeichnet, dass** die Ausfällung des Polyurethan in Schritt c) in einem Wasser enthaltenden Bad oder bei Verwendung einer Temperatur im Bereich von 80 bis 120°C erfolgt.

10. Beschichtetes Textil, erhältlich durch ein Verfahren nach den Ansprüchen 1 bis 9.

11. Beschichtetes Textil nach Anspruch 10, **dadurch gekennzeichnet, dass** es sich bei dem beschichteten Textil um Kunstleder handelt.

## Revendications

1. Procédé de fabrication de textiles enduits, consistant au moins à :
a) mettre un substrat textile en contact avec une dispersion aqueuse A comprenant au moins un sel inorganique et au moins une cellulose modifiée,
b) mettre un substrat textile en contact avec une dispersion aqueuse B comprenant du polyuréthane et
c) précipiter le polyuréthane dans ou sur le substrat textile.

2. Procédé selon la revendication 1, dans lequel le sel inorganique est un sel sélectionné dans le groupe constitué de sels de métaux alcalins et de sels de métaux alcalino-terreux.

3. Procédé selon la revendication 2, dans lequel le sel de métal alcalin est un sel sélectionné dans le groupe constitué d'halogénures de métaux alcalins, de nitrates de métaux alcalins, de phosphates de métaux alcalins, de sulfates de métaux alcalins, de carbonates de métaux alcalins et d'hydrogénocarbonates de métaux alcalins.

4. Procédé selon la revendication 2, dans lequel le sel de métal alcalino-terreux est un sel sélectionné dans le groupe constitué d'halogénures de métaux alcalino-terreux, de nitrates de métaux alcalino-terreux, de phosphates de métaux alcalino-terreux, de sulfates de métaux alcalinoterreux, de carbonates de métaux alcalino-terreux et d'hydrogénocarbonates de métaux alcalinoterreux.

5. Procédé selon la revendication 1, dans lequel le sel inorganique est présent dans la dispersion A dans une quantité de 0,01 % à 25 % en poids, relativement à la quantité totale de dispersion A.

6. Procédé selon la revendication 1, dans lequel la cellulose modifiée est un composé sélectionné dans le groupe constitué de la méthylcellulose, de l'éthylcellulose, de la propylcellulose, de l'hydroxyméthylcellulose, de l'hydroxyéthylcellulose, de l'hydroxypropylcellulose, de l'hydroxypropylméthylcellulose, de la carboxyméthylcellulose, de la carboxyéthylcellulose et de la carboxypropylcellulose.

7. Procédé selon la revendication 1, dans lequel la cellulose modifiée est présente dans la dispersion A dans une quantité de 10 ppm à 5 % en poids, relativement à la quantité totale de dispersion A.

8. Procédé selon la revendication 1, **caractérisé en ce que** le substrat textile employé est un tissu tissé, un tissu tricoté ou un non-tissé à base de fibres naturelles et/ou synthétiques.

9. Procédé selon la revendication 1, **caractérisé en ce que** le polyuréthane est précipité à l'étape c) dans un bain contenant de l'eau ou en utilisant une température de 80 °C à 120 °C.

10. Textile enduit pouvant être obtenu par un procédé selon les revendications 1 à 9.

11. Textile enduit selon la revendication 10, **caractérisé en ce que** le textile enduit est un cuir synthétique.
